

## UNITED STATES PATENT OFFICE

2,140,008

## TANNING

Ralph E. Hall, Mount Lebanon, Pa., assignor to  
 Hall Laboratories, Inc., Pittsburgh, Pa., a corporation of Pennsylvania

No Drawing. Application June 18, 1936, Serial  
 No. 85,963. Renewed February 2, 1938

## 8 Claims. (Cl. 149—5)

This invention relates to tanning, and more particularly to the prevention of discoloration by iron compounds in tanning processes and to the speeding up and increase in the efficiency of the 5 tanning operation.

The present application is a continuation-in-part of my application Serial No. 685,754, filed August 18, 1933.

Iron combines with tanning bodies to form dark 10 colored compounds which, if present in the tanning liquors or materials to be tanned, cause discoloration in the tanned materials. The waste liquors from paper making processes contain tannin bodies, sometimes called "pseudo 15 tannins". These liquors, particularly the waste sulphite liquors, are employed for tanning purposes. The waste liquors are usually treated and concentrated to form tanning compounds in the form of solid bodies or extracts. In the 20 production of such waste liquors in the paper mills, they are frequently contaminated with small amounts of iron impurities which combine with the tanning bodies in the liquors to form dark colored compounds which discolor the leather being tanned.

25 I have found that such discoloration may be prevented by employing an alkali-metal hexametaphosphate, for example sodium hexametaphosphate, in such iron contaminated tanning liquors. The hexametaphosphates have the singular property of converting the iron into soluble, very slightly ionized form, thereby preventing the iron from combining with the tanning bodies to produce the dark discolorations. The effect of the hexametaphosphates is to 30 sequester the iron in soluble, slightly ionized complexes.

35 Sodium hexametaphosphate probably has a molecular constitution indicated by the formula  $Na_2(Na_4P_6O_{18})$ . Ferrous iron combines with the hexametaphosphate to produce a but slightly ionized complex molecule believed to have the molecular constitution indicated by  $Na_2(Fe_2P_6O_{18})$ , which is initially ionized according to the 40 ionic equation,  $Na_2Fe_2P_6O_{18} \rightleftharpoons 2Na^+ + Fe_2P_6O_{18}$ , in which the radical  $Fe_2P_6O_{18}$  is very slightly ionized.

45 Similarly, ferric iron combines with sodium hexametaphosphate to form a complex from which the iron is but slightly ionized. There is evidence indicating that ferric iron forms a compound  $Na_8(Fe_4P_18O_{54})$  which is initially ionized according to the ionic equation,



50 in which the radical  $Fe_4P_18O_{54}$  is very slightly ionized.

55 As indicated by these formulae, the effect of the hexametaphosphate is to sequester the iron in the form of but very slightly ionized complexes, so that the solution has exceedingly low

ionic concentration of iron. This ionic concentration is smaller than the concentration of ionic iron in equilibrium with the tanning bodies, and accordingly, the iron will remain in solution and will not combine with the tanning bodies to form 5 the dark discoloring compounds. Since the amount of iron in the tanning liquors is usually relatively small, only a small amount of the hexametaphosphate need be ordinarily used. It is preferred to add the sodium hexametaphosphate 10 in some excess of that theoretically required, to combine with iron according to the above formulas. I have found that an amount of sodium hexametaphosphate of about 16 to 17 times that of the weight of the iron present will 15 hold the iron against discoloring combination with the tanning bodies in tanning liquors having a pH value of not over about 6 to 7. An increase in pH value results in a sharp increase in the amount of metaphosphate required until 20 at a pH value of over about 8 the metaphosphate no longer so holds the iron.

25 Fortunately, the pH values of the tanning liquors lie within the limits within which the hexametaphosphates can effectively repress the iron. Usually, an excess somewhat above these amounts is employed as a safeguard, which is not objectionable since only a small amount of the hexametaphosphate usually need be added because the amount of iron impurities is usually 30 relatively low.

35 The hexametaphosphate may be added to the waste liquors from the paper making operations during the preparation of these liquors for the tanning industry, and a compound, either as a solid or as an extract, furnished to the tanner containing sufficient hexametaphosphate to counteract such iron impurities as may be present in such tanning compound. Or the tanner may add the hexametaphosphate to the tanning liquor 40 in the tanning vats.

45 The hexametaphosphate may be employed with the natural tanning liquors, such as those produced from bark or wood, and will serve to prevent discoloration due to iron compounds which may be present in the water, the tanning compounds or the leathers to be tanned.

50 Since iron forms dark colored compounds with the pseudo tannin bodies such as are present in the waste liquors from paper making, as well as the tannins proper, when I speak of tanning liquors or tanning bodies, I intend to include the pseudo tannins as well as the tannins proper.

55 The use of alkali-metal hexametaphosphates in tanning serves other important functions in addition to preventing discoloration by iron compounds. One of the principal difficulties associated with tanning is the appearance of calcium soaps on the surface of the leather. These calcium soaps come from within the hide, being 60

- formed during the liming process. The hexametaphosphates have the property of dissolving these calcium soaps, thereby allowing the tanning liquor to act more effectively on the leather.
- 5 Even though hides which have been limed are washed before the tanning operation, the removal of calcium is frequently incomplete. In such cases the lime soaps which have been formed by the reaction between the lime and the fats
- 10 naturally present in the raw hides are not entirely removed before tanning. This frequently results in defects in the tanned hide called "spewing" which consists in the appearance of grease spots on the surface of the leather, causing
- 15 trouble in the further finishing operations. This spewing may be prevented by the use of alkali-metal hexametaphosphates in the tanning liquor due to the fact that the hexametaphosphates have the property of dissolving the lime soaps.
- 20 Lime soaps, if present, not only cause defects in the finished leather, but prevent the effective penetration of the tanning compound into the pores of the hide.
- The speed and efficiency of penetration of the
- 25 tanning liquor into the hides is increased by employing an alkali-metal hexametaphosphate in the tanning solution. The tanning of leather is commonly carried out at pH values below 5.0. At such low pH values, alkali-metal hexameta-
- 30 phosphates have the property of reacting with albumen to precipitate it and of reacting with other proteins commonly present in hides. It is believed that the effect of the hexametaphosphate in the tanning of leather rests in part at least
- 35 upon the specific reactivity between the protein constituents of the hide and the hexametaphosphate. It is generally believed that during the process of tanning, addition compounds are formed by the tannins present in the tanning
- 40 liquor and the protein constituents of the hides. Alkali-metal hexametaphosphates form insoluble addition compounds with soluble proteins, such as albumen, and insoluble proteins as well, and it is believed therefore that the presence of sodium hexametaphosphate, for example, in a tanning liquor facilitates the tanning and curing of the hide and improves the finished leather by reacting with the albumen and other proteins present in the hide. One of the most distinctive re-
- 45 actions of sodium hexametaphosphate, and in fact the method used for its qualitative detection in the presence of other phosphates, is its precipitating action on albumens in acetic acid solution. When to an acetic acid solution of egg white there is added a dilute solution of sodium hexametaphosphate, the albumen is quickly coagulated. This effect is not produced by sodium

orthophosphate or sodium pyrophosphate. It is believed that in tanning operations where sodium hexametaphosphate is employed in tanning solutions having pH values below 5.0, it reacts with the albumen and proteins present in the hide to form addition compounds, thereby increasing the speed of penetration and effectiveness of the tannin bodies.

Normal sodium hexametaphosphate has a pH value in solution of about 6 and may be advantageously used as such in the tanning liquors. In general, the normal salts, the acid salts or even the acid may be used depending upon the pH value desired and the control of the pH value in the tanning liquors. The term "alkali-metal hexametaphosphate" when used without other qualification is intended to include the acid salts as well as the normal salts.

While I prefer to use sodium hexametaphosphate because of its greater cheapness and availability, the hexametaphosphates of the other alkali-metals may be employed, such for example as the salts of potassium, ammonium, lithium, etc.

I have described the preferred procedure in carrying out the invention and have set forth what I believe to be the correct theoretical explanation of the reactions involved. It is to be understood, however, that the invention is not limited to such preferred procedure or by such theoretical explanations, but that the invention may be otherwise embodied or practiced within the scope of the following claims.

I claim:

1. A process of tanning, which comprises subjecting the materials to be tanned to a tanning liquor containing an alkali-metal hexametaphosphate.
2. A process of tanning, which comprises subjecting the materials to be tanned to a tanning liquor containing sodium hexametaphosphate.
3. A tanning liquor containing an alkali-metal hexametaphosphate.
4. A tanning liquor containing sodium hexametaphosphate.
5. A tanning preparation containing an alkali-metal hexametaphosphate.
6. A tanning preparation comprising tannin-bearing extracts and sodium metaphosphate.
7. A process for tanning hides comprising immersing hides in a bath of tannin extract and a soluble dehydrated alkali metal metaphosphate.
8. A process for tanning hides comprising immersing hides in a bath of tannin extract and a soluble sodium metaphosphate.

RALPH E. HALL.